

1

3,164,505  
GELLING OF HYDRAZINE

Paul Y. Hsieh and James V. Cartmell, Dayton, Ohio,  
assignors to The National Cash Register Company,  
Dayton, Ohio, a corporation of Maryland  
No Drawing. Filed Oct. 25, 1962, Ser. No. 233,153

8 Claims. (Cl. 149—36)

This invention relates to gelled fuel compositions and to a method for making such gels. More specifically, it relates to a semi-rigid to rigid gelled fuel composition comprising a major proportion of substantially anhydrous hydrazine and a minor proportion of a fatty acid ester of a polyol as a gelling agent.

Hydrazine is a well-known and commercially-available chemical compound and has been widely used in both industry and research. For example, it is useful as an intermediate in the manufacture of many industrially-important chemicals such as, for example, agricultural, textile, photographic, and other chemicals. Hydrazine is also important in the manufacture of explosives and as an essential ingredient in many industrially-important processes. In addition to the above-mentioned uses for hydrazine, it is a powerful and efficient fuel for rocket and jet engines. Because of its low molecular weight and high heat of combustion, hydrazine provides high energy output per unit weight.

When the gelled hydrazine composition of the invention is burned in air or in oxygen, it provides the same energy output per unit weight obtained with normally liquid untreated hydrazine.

For reasons apparent to those skilled in the art, many advantages inhere in the use of solid, rigid, or semi-rigid fuels instead of liquid fuels for jet and rocket propulsion.

In accordance with the present invention, hydrazine, which normally is liquid at room temperature (having a melting point of 2 degrees centigrade and a boiling point of 113 degrees centigrade), is readily and efficiently converted to a self-supporting rigid or semi-rigid mass, in a form suitable for use as a rocket fuel, by simply mixing a minor amount of an ester or of esters of certain fatty acids and polyols, which are specified hereinafter, with said hydrazine, and allowing the mixture to gel at room temperature, either with or without agitation.

Thus, a prime object of the invention is to provide a gelled composition comprising hydrazine and an ester of selected fatty acids and polyols.

Another object is to provide a simple and efficient process for making a gelled hydrazine composition which is self-supporting and has a consistency ranging from semi-rigid to rigid.

A further object is to provide a gelled hydrazine fuel composition having the same burning characteristics as untreated or ungelled hydrazine.

Yet another object is to provide a hydrazine composition gelled with a minor amount of a fatty acid ester of a polyol, the resulting composition having a greatly reduced hydrazine vapor pressure when compared to the vapor pressure of pure hydrazine.

These and other objects of the invention are achieved by a substantially anhydrous, self-supporting, gelled fuel composition comprising:

- (1) A major amount of hydrazine, and
- (2) A minor amount of fatty acid ester selected from the group consisting of:
  - (a) fatty acid esters of sorbitan selected from the group consisting of the monooleate, dioleate, trioleate, monostearate, and monopalmitate ester of sorbitan,
  - (b) fatty acid esters of polyethylene glycol

2

selected from the group consisting of the monooleate and the dilaurate ester of polyethylene glycol, said polyethylene glycol being liquid at room temperature and having an average molecular weight range from 200 to 600, and

(c) mixture of fatty acid esters in (a) and (b).

The following example demonstrates a preferred method for preparing gelled hydrazine according to the invention:

Three (3) grams of sorbitan monooleate (Span 80) was rapidly added to ninety-seven (97) grams of anhydrous hydrazine (95+%) maintained at room temperature in a suitable container, the contents being stirred during the addition. The time required for adding the sorbitan monooleate ester was about two (2) seconds. Immediately after the addition, the stirring was stopped, and the ester diffused very rapidly into the hydrazine to produce an opaque gel having a slightly yellow tint. Within two (2) minutes, a rigid, well-set, non-pourable gel had formed. No change in temperature was noted during the gelling operation.

The amount of ester which may be used for making the gelled hydrazine composition is not critical so long as at least a minor amount of the ester based on the total weight of ester and hydrazine is present; however, amounts of ester up to ten (10) percent are preferred. Gelled hydrazine-ester compositions having optimum characteristics are generally obtained with three (3) percent, by weight, of the ester.

It has been found that the consistency of the gel, which may range from soft and pourable to semi-rigid or rigid and non-pourable, is directly proportional to the ester concentration. The higher the concentration, the more rigid the gel. However, for any given consistency, the gelling time required for the gel to reach said consistency is a function of the specific ester and, to a lesser extent, also a function of the concentration of said ester.

The general relationship between the type of ester used as gelling agent and the time of gelling will be apparent from the following table:

| Percent | Agent                                  | Approximate gelling time vs. concentration of ester gelling agents <sup>1</sup> |                |          |
|---------|----------------------------------------|---------------------------------------------------------------------------------|----------------|----------|
|         |                                        | 1%                                                                              | 3%             | 10%      |
| 50      | 1. Sorbitan monooleate <sup>1</sup>    | 10 minutes                                                                      | 2 to 5 minutes | 1 minute |
|         | 2. Sorbitan dioleate <sup>1</sup>      |                                                                                 |                |          |
|         | 3. Sorbitan trioleate <sup>1</sup>     |                                                                                 |                |          |
|         | 4. Sorbitan monostearate <sup>1</sup>  |                                                                                 |                |          |
|         | 5. Sorbitan monopalmitate <sup>1</sup> |                                                                                 |                |          |
|         | 6. Polyethylene glycol monooleate      | Approximately one hour at 3% to 10% concentration                               |                |          |
|         | 7. Polyethylene glycol dilaurate       |                                                                                 |                |          |

<sup>1</sup> Compounds sold under the trademark "Span."

<sup>2</sup> Time required to reach maximum consistency.

Concentrations are given in percent by weight based on the total composition weight unless otherwise indicated.

From the above table it can be seen that the rate at which hydrazine gels with sorbitan esters is more rapid than with polyethylene glycol esters and that, for all practical purposes, when the latter is used as gelling agent, the rate of gelling is substantially independent of ester concentration between 3 percent and 10 percent ester.

When a sorbitan ester is the gelling agent, an increase or decrease in the concentration of said agent by a factor of ten decreases or increases the gelling time to maximum consistency by a factor of about 10, respectively. Hence, the gelling rate is directly proportional to the concentration in the range of 1 percent to 10 percent gelling agent.

No satisfactory theory or mechanism has been found to explain the instantly-described and claimed gelling

action. However, the action apparently is highly specific in nature, since, from among a large number of surface-active compounds tested, only the above-specified compounds were effective as gelling agents for hydrazine.

It will be understood by those skilled in the art that hydrazine, as well as other solid and liquid rocket propellants, are customarily utilized with oxidizers. Thus, it should be apparent that the gelled hydrazine compositions of the invention may comprise, preferably in minor proportion, such conventional oxidizers as, for example, nitric acid, oxygen progenitors such as ammonium nitrate, potassium perchlorate, etc., oxygen, and nitrogen tetroxide. Some fuel and oxidizer combinations are known to be hypergolic, and the two must, of necessity, be maintained out of contact with each other until it is desired to initiate the combustion. However, in fuel-and-oxidizer combinations which are not hypergolic, the oxidizer may be blended directly with the constituents for forming the gelled hydrazine composition.

In addition to providing hydrazine in a semi-rigid or rigid form suitable for use as a jet and rocket fuel propellant, gelled hydrazine, as described herein, overcomes several recognized problems and disadvantages associated with the storage, handling, and shipping of the normally-liquid hydrazine. Since hydrazine vapor is highly toxic and corrosive, particularly to the eyes, and forms explosive mixtures with air, it has been customary in the past to store and ship hydrazine in strong metal or glass containers. Heretofore, it was not feasible to use flexible and non-flexible polymeric and other conventional packaging materials for the storage or shipment of hydrazine, because a number of such materials were reactive with hydrazine, while others were not sufficiently impermeable to hydrazine, in either liquid or vapor state, to provide a safe level of protection. It has now been found that, at room temperature, gelled hydrazine compositions prepared according to the invention have approximately one sixth ( $\frac{1}{6}$ ) the hydrazine vapor pressure of untreated hydrazine at the same temperature. Because of this characteristic, gelled hydrazine of the invention can now be packaged, stored, and shipped in containers fabricated from unreactive packaging materials, such as flexible polymeric materials and other conventional materials, as well as in the metal and glass containers required in the past.

Although the invention is described above in terms of certain materials and embodiments, it should be understood that it is susceptible to changes without departing from the scope of the invention as described in the following claims.

What is claimed is:

1. A substantially anhydrous, self-supporting, gelled fuel composition comprising:

(1) A major amount of hydrazine, and  
(2) A minor amount of fatty acid ester selected from the group consisting of:

(a) fatty acid esters of sorbitan selected from the group consisting of the monooleate, dioleate, trioleate, monostearate, and monopalmitate ester of sorbitan,

(b) fatty acid esters of polyethylene glycol selected from the group consisting of the monostearate and the dilaurate ester of polyethylene glycol, said polyethylene glycol being liquid at room temperature and having an average molecular weight range from 200 to 600, and

(c) mixture of fatty acid esters in (a) and (b).

2. The composition of claim 1 wherein said composition comprises:

(1) at least 90 percent, by weight, hydrazine, and  
(2) up to 10 percent, by weight, of the ester, the percentages based on the total weight of hydrazine and ester.

3. The composition of claim 1 wherein the ester is sorbitan monooleate.

4. The composition of claim 1 wherein the ester is sorbitan dioleate.

5. The composition of claim 1 wherein the ester is sorbitan trioleate.

6. The composition of claim 1 wherein the ester is polyethylene glycol monostearate.

7. The composition of claim 1 wherein said composition comprises:

(1) 97 percent, by weight, hydrazine, and  
(2) 3 percent, by weight, of the ester, the percentages based on the total weight of hydrazine and ester.

8. The method of converting normally liquid substantially anhydrous hydrazine to a firm self-supporting gel which comprises dissolving in said anhydrous hydrazine, with little or no agitation, at room temperature, a minor amount of a fatty acid ester of a polyol selected from the group consisting of sorbitan monooleate, sorbitan dioleate, sorbitan trioleate, sorbitan monostearate, sorbitan monopalmitate, polyethylene glycol monostearate, and polyethylene glycol dilaurate, and allowing the mixture to gel while at room temperature.

#### References Cited in the file of this patent

#### UNITED STATES PATENTS

|    |           |                |               |
|----|-----------|----------------|---------------|
| 50 | 3,021,667 | Griffin et al. | Feb. 20, 1962 |
|    | 3,077,072 | Rice           | Feb. 12, 1963 |